

# UNITED STATES PATENT OFFICE.

WILLIAM A. FAIRBURN, OF SHORT HILLS, NEW JERSEY, ASSIGNOR TO THE DIAMOND MATCH COMPANY, OF CHICAGO, ILLINOIS, A CORPORATION OF ILLINOIS.

## TREATED MATCH-SPINT AND PROCESS OF PRODUCING THE SAME.

1,163,869.

Specification of Letters Patent.

Patented Jan. 18, 1916.

No Drawing.

Application filed June 1<sup>st</sup>, 1913. Serial No. 774,314.

To all whom it may concern:

Be it known that I, WILLIAM A. FAIRBURN, a citizen of the United States, and resident of Short Hills, in the county of 5 Essex and State of New Jersey, have invented certain new and useful Improvements in Treated Match-Splints and Processes of Producing the Same, of which the following is a specification.

10 The object of this invention is to provide a simple, economical and efficient process whereby flaming and non-glowing properties are imparted to match splints; and to that end I grind a powdered anti-glowing 15 substance into a heavy-bodied oleaginous substance and then incorporate the mixture with an unctuous inflammable material in the presence of heat. This mixture is preferably agitated, or kept in circulation, and 20 the match splints are then dipped into the same and impregnated therewith.

In pursuance of my invention, (which also embraces the impregnated splints) the preferred anti-glowing substance which I 25 employ is boric acid, and the preferred oleaginous substance into which it is intimately ground is a heavy-bodied petroleum product, such as petrolatum; the proportion being about, by weight, 2 parts of petro- 30 latum to 1 part of boric acid.

The preferred inflammable material to which the mixture is added is melted paraffin wax, the proportion being about 9 parts of paraffin wax to 1 part of the petrolatum- 35 boric acid mixture. The mixture, being preferably agitated or kept in circulation, is maintained at a temperature of about 250° Fahr., and the match splints are dipped thereinto and then removed. Such splints 40 are thus effectually impregnated with the constituents of the mixture and as a result the splints possess the requisite inflammable and non-glowing properties; that is to say, the paraffin serves as a vehicle to transmit the flame from the match head to the splint and the boric acid renders the splint non-glowing after the flame has been extinguished.

I do not limit my invention to the specific 50 materials or proportions herein mentioned; but

What I claim is—

1. A process of treating match splints to impart flaming and non-glowing properties thereto, which comprises grinding an anti-glowing material into a greasy, heavy bodied oleaginous substance, mixing the same with an unctuous, waxy, inflammable material in a heated condition, the melting point of said oleaginous substance being materially lower than that of said inflammable material, and dipping the splints into said mixture while said mixture is molten. 55

2. A process of treating match-splints to impart flaming and non-glowing properties thereto, which consists in grinding an anti-glowing material into a heavy-bodied oleaginous product, mixing the same with melted paraffin wax at a temperature of about 250° Fahr., and dipping the splints there- 65 into. 70

3. A process of treating match-splints to impart flaming and non-glowing properties thereto, which consists in subjecting the splints to a bath of melted paraffin with 75 which is incorporated an intimate mixture of petroliatum and an anti-glowing material.

4. A process of treating match splints to impart flaming and non-glowing properties thereto, which consists in subjecting the 80 splints to a bath of melted paraffin wax with which is incorporated a mixture comprising boric acid ground into petrolatum.

5. As a new article of manufacture, a match splint impregnated with a mixture 85 containing a waxy, unctuous, inflammable material, a heavy-bodied, greasy oleaginous substance and a finely divided anti-glowing material.

6. As a new article of manufacture, a 90 match splint impregnated with a mixture comprising paraffin wax, petrolatum and finely divided boric acid.

Signed at New York in the county and State of New York, this 16th day of June 95 A. D. 1913.

WILLIAM A. FAIRBURN.

Witnesses:

B. CHANDLER SNEAD,  
FRANCES R. GRIFFIN.